

July 21, 1936.

J. PAGE

2,047,982

WALLBOARD JOINT

Filed Sept. 13, 1934

Fig. 1



Fig. 2



Fig. 3



Fig. 4



Fig. 5



INVENTOR  
JOHN PAGE

BY  
L.A. Paley  
ATTORNEY

## UNITED STATES PATENT OFFICE

2,047,982

## WALLBOARD JOINT

John Page, Evanston, Ill., assignor to United States Gypsum Company, Chicago, Ill., a corporation of Illinois

Application September 13, 1934, Serial No. 743,847

7 Claims. (Cl. 72—16)

This invention relates to building constructions and has reference more particularly to wallboard joints and their method of preparation.

In the history of the building industry, various proposals have been made for treating the joints of wallboards when attached to studs with their edges abutting. One of these joint treatments is covered in patent to Green No. 1,703,667, in which a perforated metal tape is adhesively secured over the wallboard joint, the perforations being provided to permit drying out of the adhesive and also to somewhat improve the bond of the tape to the face of the boards. The resulting joint is covered with a plastic paint, wall paper, or other decorative covering.

Cloth tapes and paper tapes have also been used. Cloth tapes have low transverse tensile strengths and high stretch so that they are apt to rupture and permit cracks to form in the decorative coatings. The same is true of the paper tapes which have heretofore been used. In addition paper tapes heretofore proposed have a high transverse and longitudinal expansion on wetting so that wrinkling due to application of adhesive prevents the tape from lying flat on the surfaces of the wallboards and also produces hair line cracks along the edges of the tape as it dries and shrinks.

In order to obtain sufficient cross tensile strength to prevent cracking at joints with ordinary papers it is necessary to use a paper of considerable thickness. This is unsatisfactory for two reasons. First, the thick tape makes a thick bulging joint which is difficult if not impossible to hide. Second, due to the excessive thickness and resultant stiffness of the tape it will not shrink down properly into depressions in the joint as the adhesive dries out. This means unbonded areas of tape over these depressions which will during painting swell slightly and form blisters. When the paint dries these blisters will not entirely straighten out and will remain as small lumps which will make the joint unsightly.

In my preferred method of application the joint is first filled flush with the surface of the board, covering nail heads, and if necessary building up low spots. After drying, the rough spots and lumps are lightly sanded off to form as even as possible a flat bed for the tape. Next,

a thick heavy bodied adhesive is applied over the filled joint. The tape is then placed over this and pressed down firmly into it. The excess adhesive is squeezed out by this pressure and is scraped off. The adhesive is made heavy for two reasons. First, to have sufficient body to hold down the edge of the tape and prevent it from curling. Second, in squeezing the excess of the heavy bodied adhesive out from under the tape the adhesive flows and fills every crevice and depression in the surface of the board, incompletely filled nail heads, etc. Then as the adhesive dries, due to its tackiness and body, it pulls the tape down into these depressions and bonds it to the board over the entire area of tape. If this type of adhesive were not used, there would be a hollow spot behind the tape over each depression. Later when dampened by water paint, the tape over this area will swell and blister. This is exactly what happened in previous tape systems where a thin adhesive or an adhesive previously applied to the back of the tape was used.

After the adhesive has dried and pulled the tape down into the depressions a finishing or feathering cement is used to fill up these depressions and feather off the edges of the tape. When dry this cement is sanded down to give a smooth even surface which when properly painted or treated with other conventional decorative materials is substantially invisible.

An object of this invention, therefore, is to provide an improved tape for application over the joints of wallboards.

Another object of the invention is to provide an improved paper tape for joint treatment which has a high modulus of elasticity, a low transverse and longitudinal expansion on wetting, a high transverse tensile strength and freedom from edge cracking when applied in a wall construction.

Another object of the invention is to produce an improved method of applying paper tape to wallboard joints.

A further object of the invention is to provide an improved wall construction embodying my improved joint tape; also to improve joint tapes and wallboard joints in other respects herein-after specified and claimed.

Reference is to be had to the accompanying

drawing forming a part of this specification, in which

Fig. 1 is a sectional perspective view of my improved wall construction embodying my improved joint tape, 5

Fig. 2 is a sectional plan view through the wall construction,

Fig. 3 is a fragmentary elevation of the form of joint tape shown in Fig. 1,

Fig. 4 is a fragmentary elevation of a modified form of joint tape, and

Fig. 5 is a sectional view through a further modified form of the joint tape.

In preparing a wall, ceiling or partition, it is customary to provide studs or joists 10 to which wallboards 11 are attached by nails 12a. The wallboards 11 are often made with a gypsum core 12 faced on both sides with paper cover sheets 13 which are folded about the edges of the core 12 to form folds 14 forming protected edges. The wallboards 11 may also be made of vegetable fibers, such as the wood fiber insulating boards which are well known to the art. The wallboards may

One of the salient features of my invention is to provide a paper tape of special characteristics which will produce a joint having a transverse tensile strength substantially equal to that of the board itself so that no cracks will be formed in the coating 18 at the joint due to expansion and contraction of the board because of changes in temperature or warping of the studs 10. This may be accomplished in part by utilizing a paper made in a paper machine which accomplishes a crossing of a substantial proportion of the fibers of which the paper is composed. This imparts to the paper a high transverse tensile strength, a low stretch, a high breaking load, and a high modulus of elasticity. The tape also has a low transverse and longitudinal expansion on wetting so that it lies perfectly flat on the wall surface during application and during the drying of the adhesive. My improved method of application of the tape also contributes in securing the above results. 10 15 20

In order to show the comparative strength of my improved tape compared to other tapes previously used, the following data is given:—

| 25 | Material                    | Thickness of tape (inches) | Cross tensile modulus of elasticity of tape, lbs./inch <sup>2</sup> | Cross tensile strength of tape, lbs./in. | Ratio cross tensile strength of tape, lbs./in. length/.001 in. thickness | Longitudinal tensile strength of tape, lbs./in. | Ratio longitudinal tensile strength of tape, lbs./in. length/.001 in. thickness | Transverse stretch of tape at breaking load, percent | 25 |
|----|-----------------------------|----------------------------|---------------------------------------------------------------------|------------------------------------------|--------------------------------------------------------------------------|-------------------------------------------------|---------------------------------------------------------------------------------|------------------------------------------------------|----|
| 30 |                             |                            |                                                                     |                                          |                                                                          |                                                 |                                                                                 |                                                      | 30 |
| 35 | Paper tape No. 1.....       | 0.045                      | 71,000                                                              | 24                                       | 5.3                                                                      | 49                                              | 10.9                                                                            | .....                                                | 35 |
|    | Paper tape No. 2.....       | 0.005                      | 50,000                                                              | 25                                       | 5.0                                                                      | 56                                              | 11.2                                                                            | .....                                                |    |
|    | Paper tape No. 3.....       | 0.007                      | 39,285                                                              | 33                                       | 4.7                                                                      | 81                                              | 11.5                                                                            | .....                                                |    |
|    | Paper tape No. 4.....       | 0.005                      | 70,000                                                              | 30                                       | 6.0                                                                      | 49                                              | 9.8                                                                             | .....                                                |    |
|    | Paper tape No. 5.....       | 0.0145                     | 129,000                                                             | 60                                       | 4.14                                                                     | 145                                             | 10.0                                                                            | .....                                                |    |
|    | Kraft wrapping paper.....   | 0.005                      | 85,000                                                              | 27                                       | 5.4                                                                      | 35                                              | 7.0                                                                             | .....                                                |    |
|    | Wallboard paper.....        | 0.021                      | 57,600                                                              | 32                                       | 1.5                                                                      | 105                                             | 5.0                                                                             | .....                                                |    |
|    | Improved paper tape.....    | 0.0095                     | 185,000                                                             | 60-81                                    | 6.3-8.4                                                                  | 144-116                                         | 15.2-12.2                                                                       | 4.5                                                  |    |
|    | Perforated metal tape.....  | 0.004                      | .....                                                               | 95                                       | .....                                                                    | .....                                           | .....                                                                           | 12.5                                                 |    |
|    | Cloth tape No. 1.....       | 0.006                      | .....                                                               | 49                                       | .....                                                                    | .....                                           | .....                                                                           | 10.0                                                 |    |
| 40 | Cloth tape No. 2 sized..... | 0.013                      | .....                                                               | 23                                       | .....                                                                    | .....                                           | .....                                                                           | 7.5                                                  | 40 |

also be the well known paper pulp boards.

In the joint between the wallboards, I preferably apply a crack filler cement having about the following composition:—

|                        | Pounds |
|------------------------|--------|
| Casein.....            | 48     |
| High calcium lime..... | 22     |
| Borax.....             | 10     |
| Mica.....              | 100    |
| Marble flour.....      | 820    |

This cement is smoothed off level with the faces of the boards and allowed to dry.

An adhesive 15 is then applied to the surface of the board over the joint, this adhesive preferably having about the following formula:

|                          | Pounds |
|--------------------------|--------|
| Casein.....              | 850    |
| Borax.....               | 42     |
| Trisodium phosphate..... | 102    |
| Tribromophenol.....      | 6      |

A variation of plus or minus 20% can be made in the amounts of ingredients in the above formulas with satisfactory results. Other mineral fillers, preservatives and casein solvents may also be used. While the adhesive 15 is still moist, a paper tape 16 is smoothed out over the joint. If an adhesive and finishing cement are used the taper is formed with the cement. The adhesive itself is thin and cannot be built up to a taper. After the adhesive is dried, a decorative coating 18 is applied to the exposed surface of the boards completely concealing the joint, this decorative coating being paint, wall paper or the like. 75

It will be noted from the above data that my improved paper tape is characterized by low stretch at breaking load, high modulus of elasticity, and high transverse and longitudinal strengths, which make it ideal as a joint tape over wallboard joints. In this connection, I consider that a paper joint tape should have a cross tensile modulus of elasticity of at least 100,000 lbs./in.<sup>2</sup>. 45 50

My improved tape is also noteworthy in its unusually low transverse and longitudinal expansion on wetting. The following data on expansion after a 2 min. immersion in water at 70° F. illustrates this point:—

|                          | Tape    | Expansion across tape | Expansion lengthwise of tape |
|--------------------------|---------|-----------------------|------------------------------|
|                          | Percent | Percent               | Percent                      |
| Improved paper tape..... | 0.78    | 0.26                  | .....                        |
| Paper tape No. 6.....    | 2.34    | 0.52                  | .....                        |
| Paper tape No. 7.....    | 2.3     | 0.5                   | .....                        |
| Paper tape No. 8.....    | 2.6     | 0.25                  | .....                        |

I consider that a paper tape should have a maximum transverse expansion on wetting of 1.5% and maximum longitudinal expansion of 0.5% in order to provide satisfactory application characteristics. 65

Of course, a high strength and low stretch at breaking load of the finished joint and its resistance to rupture due to thermal expansion and contraction and warping of the studs, are essential, and in this my improved joint system excels. 70 75

The following data shows the superiority of my joint system:—

| 5  | Joint                 | Ultimate strength  | Stretch at breaking load |
|----|-----------------------|--------------------|--------------------------|
| 10 |                       | Lbs./inch of joint | Inches                   |
| 15 | Improved joint tape   | 99                 | 0                        |
| 10 | Perforated metal tape | 82                 | 0                        |
| 15 | Cloth tape No. 1      | 76                 | 564                      |
| 20 | Cloth tape No. 2      | 50                 | 564                      |

The superior bond between the improved paper tape and the wallboards is partly responsible for the superior strength of the resulting joint.

In addition to the advantages of the improved joint as above set forth, I have so formed the edges of the paper tape, that all cracking of the decorative coating at the edges of the tape has been practically eliminated. In the form of tape shown in Figs. 1 and 3, the edges of the tape have been serrated to provide irregular saw tooth projections 20. These projections 20 distribute the load at the edges of the tape where danger of rupture between the tape and feathering cement or wall finish is greatest. In the form of tape shown in Fig. 4, the edges of the tape are irregular by wavy projections 21 which may be formed by cutting or tearing. Tearing of the edges can be accomplished by saw tooth rolls instead of the conventional roll and knife. In the form of tape shown in Fig. 5, bevels 22 are formed on the edges of the tape which serve to secure a better adhesion between the edges of the tape and the faces of the wallboards, as well as permitting a better feathering out of the overlying cement and decorative coating to form a smooth and invisible joint. These edge treatments combined with other advantageous characteristics of the improved tape, provide a crackless and smooth joint not heretofore obtained.

I would state in conclusion, that while the examples described constitute practical embodiments of my invention, I do not wish to limit myself precisely to these details since manifestly, the same can be considerably varied without departing from the spirit of the invention as defined in the appended claims.

Having thus described my invention, I claim as new and desire to secure by Letters Patent:—

1. A paper tape suitable for adhesive attachment to wallboard joints, comprising a strip of paper having a substantial proportion of crossed fibers extending transversely of said strip, the

longitudinal edge portions of said strip of paper being weaker than the central portions thereof to retard the formation of edge cracks along said tape when applied to said wallboard joint.

2. In a wallboard construction, the combination with wallboard having the edges thereof attached to supporting framework in substantially abutting relation to form a wallboard joint, of a strip of thin paper tape adhered thereto having a large portion of its fibers extending transversely of said joint.

3. In a wallboard construction, the combination with wallboard having the edges thereof attached to supporting framework in substantially abutting relation to form a wallboard joint, of a strip of paper tape adhered thereto in which a large proportion of the fibers extends transversely of the tape and of the joint, the edge portions of the tape being weaker than the central portions thereof.

4. In a wallboard construction, the combination with wallboard having the edges thereof attached to supporting framework in substantially abutting relation to form a wallboard joint, of a strip of paper tape adhered thereto in which a large proportion of the fibers extends transversely of the tape and of the joint, the edges of the tape being feathered so as to retard the formation of edge cracks along the tape edges.

5. In a wallboard construction, the combination with wallboard having the edges thereof attached to supporting framework in substantially abutting relation to form a wallboard joint, of a strip of paper tape adhered thereto in which a large proportion of the fibers extends transversely of the tape and of the joint, the edges of the tape being serrated so as to retard the formation of edge cracks along the tape edges.

6. In a wallboard construction, the combination with wallboard having the edges thereof attached to supporting framework in substantially abutting relation to form a wallboard joint, of a strip of paper tape adhered thereto in which a large proportion of the fibers extends transversely of the tape and of the joint, the edges of which tape being sufficiently irregular to retard the formation of edge cracks along the tape edges, the tape having a minimum cross tensile modulus of elasticity of 100,000 pounds per square inch.

7. A wallboard construction as in claim 2 in which the tape is not substantially thicker than 0.01 inch.

JOHN PAGE. 55

CERTIFICATE OF CORRECTION.

Patent No. 2,047,982.

July 21, 1936.

JOHN PAGE.

It is hereby certified that error appears in the printed specification of the above numbered patent requiring correction as follows: Page 3, second column, line 37, claim 5, for the word "point" read joint; and that the said Letters Patent should be read with this correction therein that the same may conform to the record of the case in the Patent Office.

Signed and sealed this 15th day of September, A. D. 1936.

Henry Van Arsdale